

## UNITED STATES PATENT OFFICE

2,343,158

SPATTER AND CLEANING SHIELD FOR  
ELECTRIC ARC WELDING

Frank W. Scott, Minneapolis, Minn., assignor to  
Marquette Manufacturing Co., Inc., Minneapolis, Minn., a corporation of Minnesota

No Drawing. Application January 12, 1942,  
Serial No. 426,500

5 Claims. (CL 166-2)

My invention relates to a shield for the portion of metal adjacent the position where an electric weld is to be made by the arc method.

One object of the invention is to provide a shield in the form of a solution of substantially paint-like consistency, which may be applied by a paint brush to the metal adjacent the portion to be welded, the shield thereupon preventing the spray or spatter of molten metal and slag from the welding operation being deposited at undesirable points on the metal.

In connection with the welding of metals by means of the electric arc the welding process is accompanied by a spray or spatter of molten metal and slag from the point where the weld rod and the metal being welded make contact. This spray or spatter of molten metal and slag fuses onto the metal being welded and requires considerable time and effort for its removal.

The primary object of the present invention is the provision of a protective coating of fire-proof substance that prevents spray or spatter of molten metal and slag from sticking to the metal being welded.

Another object of the invention is to provide a spatter shield which may be applied in the form of a thin layer or coating to the metal, the nature of the spatter shield being such that the electric arc is rendered more stable and the physical character of the weld metal is improved, the shield being readily removable after the welding operation is completed and carrying with it the small particles of metal and slag that would otherwise have fused onto the metal being welded.

Still a further object is to provide a mixture of certain ingredients which may be sold dry to the user and mixed by him with water to the desired consistency, transportation costs thereby being reduced due to the absence of the water from the ingredients during shipping.

Another object is to provide a protective coating having as its principal ingredient asbestos whereby the coating or shield is unaffected by fire, and, due to its fibrous structure, forms a mat to hold the spatter of molten metal so that the mat and spatter can be removed after the completion of the welding operation.

With these and other objects in view my invention consists in the provision of certain ingredients in combination with each other whereby the objects contemplated are attained, as hereinafter more fully set forth and pointed out in my appended claims. Although the invention is susceptible of variation in the propor-

tions of the ingredients and in the number and character of the ingredients used, it is unnecessary to fully describe more than one representative composition suitable for spatter shield purposes, with reference being made to certain variations in the combination of ingredients, some of which may be omitted where unnecessary. The purpose of the following specification is, therefore, to give a full understanding of the invention, both from its constitutional and functional standpoint, and in accordance therewith I have described a desirable embodiment of the invention.

The principal ingredient of my spatter shield or protective coating is asbestos. Asbestos is a broad term, as it applies to a kind of material unaffected by fire. Such material may be a silicate of magnesia and/or lime, and one or more other metals, as iron, manganese, etc. Asbestos has various mineralogical classifications, as amphibole, amianthus, chrysotile, serpentine and pyroxene groups of minerals. The use of the general term asbestos, as used in the following specification, is understood to include all these varieties of mineral silicates.

Asbestos is characterized by its fibrous structure. When finely ground and mixed with a sufficient quantity of water to form a slurry or solution of paint-like consistency, the composition may be applied as a protective coating against weld metal spatter, the fibers thereupon matting together to form a tough, coherent shield that is not penetrated by the molten particles as they are projected from the weld being made. After welding, this mat holding the spatter is easily brushed off or stripped from the surface of the metal.

Asbestos fiber alone, even when ground finely, does not form a suspension in water, but settles rapidly from the slurry formed by mixing water and asbestos together. To prevent this settling, a permanent suspension may be made by the use of certain bentonites. Bentonite is a rock that contains substantially 75 percent or more of the crystalline, clay-like minerals, montmorillonite or beidellite. The bentonite that is most suitable for my spatter shield composition has a strong affinity for water, absorbs several times its weight, or as much as ten or more times its volume of water, with a constant increase in volume (which may be ten or more times the original volume). This bentonite thus forms a slippery, plastic, gelatinous mass that resembles soft soap and holds the finely divided asbestos in an ideal condition.

for application, as by a paint brush or the like, to the metal surface.

In addition to the asbestos and bentonite, I have found it convenient, and often necessary, to use certain proportions of a cleaning composition such as borax or sodium borate, mixed with the asbestos, bentonite and water. In many cases, the metal being welded is dirty and oily or greasy, so that the hydrous slurry does not spread evenly over the surface of the metal. The borax or sodium borate acts to clean the metal, to remove the grease and dirt and permits a smooth, even coating of asbestos and bentonite to be applied. This cleansing action of the borax is in addition to the detergent action of bentonite itself. Bentonite, in cleansing, seems to promote emulsions. It absorbs dirt (both solid and liquid) and prevents its return to the metal surface. The use of borax with the bentonite effectively cleans the metal surface, allows the protective film to spread evenly on the metal surface and thus gives perfect protection.

In addition to the asbestos and bentonite, I have found that the use of borax or sodium borate, besides acting as a cleaning agent in the protective coating, aids or improves the stability of the electric arc and improves the soundness of the weld metal deposited. The presence of the alkali vapor in the electric arc lowers the electrical resistance of the air or gas, thus stabilizing the arc itself. This is of particular value when alternating current welding is being done. The smoother the arc action, the better the weld itself will be. For this reason, borax or sodium borate is to be considered a desirable ingredient in my protective coating.

Borax or sodium borate in the protective coating also improves the appearance and strength of the weld metal. The flux on a weld rod forms a slag as the metal is deposited and covers the weld metal as a protective film. At times this slag interferes with the smooth flow of the weld metal itself, because the slag has a high temperature freezing point. It may even solidify along the edges of the weld metal before the weld metal itself is solidified. This results in a convex bead and in entrapped slag in the weld. Also, the wavy line on the surface of the weld metal bead may be very deep and entrap slag. The addition of asbestos, the bentonite, and particularly borax, to the slag, lowers the fusing point of the slag formed by the flux on the rod. This permits the weld metal to flow more freely and tends to produce very fine-waved beads of excellent appearance. The fluxing action of the borax produces stronger and cleaner welds.

Due to the cleaning action of borax or sodium borate on the metal adjacent the weld, and due to improving the stability of the electric arc, as well as improving the appearance and strength of the weld metal, I have found that borax or sodium borate, whether applied in solution, as a solid or as a paste, by itself is desirable as a spatter and cleaning shield for electric arc welding. In other words, the borax or sodium borate may be used alone, or in combination with asbestos and/or bentonite to obtain various desirable results.

In addition to asbestos, bentonite and borax, I have found that the addition of finely divided graphite to my spatter shield composition gives the shield coating greater smoothness in the application to the metal, and better covering power. I have also found that the stability of the electric arc is also increased through the addition

of finely divided graphite. As in the case of borax, the stability of the arc gives a more sound and stronger joint in the weld metal itself, as well as improving the appearance of the joint. For these reasons, graphite may be considered desirable in the protective coating. If, however, the presence of carbon is detrimental to the work being done, the graphite can be omitted without decreasing the power of the coating for preventing the striking of weld metal spatter to the metal being welded.

The proportions of the foregoing described ingredients may be varied rather widely to secure the desired results and attain the objects contemplated. It is to be understood that my claims are not to be limited to a particular analysis, as many proportions of the ingredients give outstanding results. By way of example, I submit the following formula for producing a mixture having exceptionally good, all-around properties. The percentages shown are based upon weight.

Ingredient:

|           | Per cent         |
|-----------|------------------|
| Asbestos  | Substantially 75 |
| Bentonite | Substantially 9  |
| Borax     | Substantially 8  |
| Graphite  | Substantially 8  |

The foregoing ingredients are then mixed with the proper amount of water to form a smooth, paint-like slurry. Depending upon variations in the characteristics of the dry ingredients and upon the consistency of coating desired by the operator, the amount of water may be varied. In most cases, I find 5.6 parts, by weight, of dry ingredients and 8.3 parts, by weight, of water, suitable. The resulting slurry is applied by means of a brush or other suitable means to the seam being welded, and on both sides of the seam, as far as the spatter may be objectionable. Welding may be done at once, or the coating may be allowed to dry before the welding is begun. It will be found that the coating will be an effective shield for preventing any sticking of weld metal spatter and the shield may be readily stripped from the metal after the welding process has been completed. Any powder deposit remaining may be readily brushed off with a dry brush, and the metal does not require any washing, as with certain clay-like types of spatter shields now on the market.

In accordance with the provisions of the patent statutes, I have described a composition suitable for use as a spatter shield, described the principle of operation and use thereof, and have supplied a formula for the mixture in accordance with my invention. I consider the foregoing specification to represent the best embodiments thereof, but I desire to have it understood that the ingredients disclosed, as well as the proportions thereof, are only illustrative, and that the invention may be carried out by equivalents which may be reasonably included with the scope of the appended claims without sacrificing any of the advantages of the invention.

What I claim as my invention and desire to secure by Letters Patent of the United States is:

1. A spatter and cleaning shield for electric arc welding comprising asbestos, bentonite, borax and graphite mixed with sufficient water to form a slurry of paint-like consistency.

2. A spatter and cleaning shield for electric arc welding comprising a slurry formed of asbestos, bentonite, borax, graphite and water, the asbestos being predominant.

3. A spatter and cleaning shield for electric arc welding comprising a composition of asbestos and borax, the predominant ingredients being asbestos.

4. A spatter and cleaning shield for electric arc welding comprising a slurry containing the following ingredients: substantially three-fourths asbestos and equal parts of bentonite, borax and graphite, the foregoing ingredients

being mixed with sufficient water to form a paint-like slurry to be applied to the metal adjacent the portion thereof to be welded.

5. A spatter shield for electric welding comprising a composition of substantially three-fourths asbestos and equal parts of bentonite, borax and graphite.

FRANK W. SCOTT.